# EUROPEAN PATENT SPECIFICATION

(11) **EP 0 543 921 B1**
(45) Date of publication and mention of the grant of the patent: **08.03.1995**
(21) Application number: 91915799.0
(22) Date of filing: 09.08.1991
(51) Int. Cl.: G03C 7/30

(54) **PHOTOGRAPHIC MATERIAL**
PHOTOGRAPHISCHES MATERIAL
MATERIAU PHOTOGRAPHIQUE

(30) Priority: 16.08.1990 US 568398
(43) Date of publication of application: 02.06.1993
(73) Proprietor: EASTMAN KODAK COMPANY, Rochester, New York 14650-2201 (US)
(72) Inventor: NELSON, John, Victor, Penfield, NY 14526 (US); BOWNE, Arlyce, Tolman, Rochester, NY 14612 (US)
(74) Representative: Brandes, Jürgen, Dr.
(86) International application number: US9105673
(87) International publication number: WO9203762

(56) References cited:
- EP-A- 0 326 406
- EP-A- 0 327 274
- EP-A- 0 338 785
- EP-A- 0 368 356

## Description

### Field of the Invention

This invention relates to photography and to radiation-sensitive silver halide photographic materials.

### Background of the Invention

Color silver halide photographic materials rely on coupler compounds to form dyes that make up the image recorded in such materials. Usually a yellow dye-forming coupler will be associated with a blue-sensitive silver halide emulsion layer, a magenta dye-forming coupler will be associated with a green-sensitive silver halide emulsion layer, and a cyan dye-forming coupler will be associated with a red-sensitive silver halide emulsion layer. These couplers will be referred to below simply as yellow couplers, magenta couplers, and cyan couplers. With color negative materials, the material is exposed to light and processed with a color developer that imagewise forms a silver image and a dye image. The silver image is formed by the color developer reducing the exposed silver halide to form silver and oxidized color developer. The dye image is formed by the reaction of oxidized color developer with dye-forming coupler. The silver image is bleached and solubilized for removal, leaving only a negative color dye image. This image is then used to expose another color negative material to form a positive color dye image.

With reversal materials, the material is generally exposed and processed with a black-and-white developer to form a negative silver image in each layer. The remaining undeveloped silver halide thus forms a positive imagewise pattern. The remaining silver halide is then fogged and processed in a color developer to form a dye image along with the silver. All the silver is then bleached and solubilized for removal, leaving only the positive color dye image.

There are many known classes of compounds that are useful as couplers in photographic materials. 5-Pyrazolone compounds and pyrazoloazole (e.g., pyrazolotriazole) compounds are well-known as magenta couplers. Such couplers are described in, for example, James, The Theory of the Photographic Process, MacMillan, 1977.

Couplers may be of the 2-equivalent or the 4-equivalent type. With 4-equivalent couplers, a hydrogen atom is cleaved from the coupler compound at the coupling position when the compound couples with the oxidized color developer. This type of coupler requires the reduction of four moles of silver halide to silver in order to form one mole of dye. With 2-equivalent couplers, a coupling-off group, such as halogen, is cleaved from the coupler compound at the coupling position during coupling with oxidized color developer. This type of coupler requires the reduction of two moles of silver halide to silver to form one mole of dye.

Exemplary photographic elements containing dye forming couplers are shown in EP A 0 362 406, EP A 0 327 274, EP A 0 338 785 and EP A 0 368 356. Among the magenta couplers contained in known photographic elements are those that can wander out of the layer in which they are coated. It has now been discovered that when such magenta couplers are used in a photographic material containing a yellow coupler having a low enough relative reactivity with oxidized developer compared to the reactivity of the magenta coupler with oxidized developer, unwanted dye can be formed as a result of reaction between magenta coupler that has wandered out of its layer and developer that has been oxidized by reaction with silver halide from the yellow coupler layer. This results in undesirable magenta contamination of the yellow record of the photographic material.

### Summary of the Invention

According to the present invention, this problem is solved, and the propensity for magenta dye contamination of the yellow record is substantially alleviated, with a color reversal photographic material comprising a support having thereon:
a magenta coupler layer that includes a silver halide emulsion and a magenta coupler compound,
a yellow coupler layer that includes a silver halide emulsion and a yellow coupler compound,
characterized in that:
the magenta coupler compound is one that is susceptible to wandering out of the layer in which it is coated,
the yellow coupler compound has a relative reactivity, as defined herein, of not greater than 0.9, and
the yellow coupler layer, or a layer between it and the magenta coupler layer, includes an oxidized developer competitor compound having a relative reaction rate, as defined herein, of at least 1.6.

Scavengers for oxidized developing agent have been placed in an interlayer between coupler containing silver halide emulsion layers (see, e.g., EP A 0 327 274 and EP A 0 338 785) to prevent oxidized developing agent generated in one layer from wandering to an adjacent layer. Such scavengers have also been coated in a coupler containing silver halide emulsion layer (see, e.g., EP A 0 326 406) to compete for oxidized developing agent with the coupler in that layer. However, neither of these situations is the same as the present invention.

### Description of the Preferred Embodiments

The magenta couplers useful in the practice of the invention can be a member of any of the known classes of couplers that are well-known in the art, as described, for example in the above-referenced James. These include both 5-pyrazolone couplers and pyrazoloazole couplers such as pyrazolotriazole couplers. In order to achieve the benefit of the invention, the magenta coupler should be one that is susceptible to wandering out of the layer in which it is coated. The degree of susceptibility to wandering that it should have, however, will vary with factors such as the reactivity of the magenta coupler with oxidized developer, the choice of yellow coupler and its reactivity with oxidized developer, the processing conditions, the concentration of the magenta coupler, and the concentration of the yellow coupler. High concentrations of the magenta coupler, low concentrations of the yellow coupler, high reactivity and/or extinction of the magenta coupler, low reactivity and/or extinction of the yellow coupler, and combinations thereof are all factors that would allow the invention to be practiced with a magenta coupler having a relatively low susceptibility to wandering compared to the situation where those factors are reversed (e.g., low concentrations of the magenta coupler, etc.).

As discussed above, the magenta coupler used in the practice of the invention can be from any class. One such class of couplers is the 5-pyrazolone class, which can be represented by the formula:
wherein
R₁ represents a carbonamido group, an arylamino (preferably anilino) group, a ureido group, a sulfonamido group, an alkylamino group, or a heterocyclic amino group,
R2 represent a substituted or unsubstituted aryl group, and
X represents hydrogen, or a group capable of being released by a coupling reaction with an oxidized aromatic primary amine developing agent. This group is hereinafter referred to as a coupling-off group. Coupling-off groups are known in the art and may include a group containing an aliphatic group, an aromatic group, a heterocyclic group, an aliphatic, aromatic, or heterocyclic sulfonyl group, or an aliphatic, aromatic, or heterocyclic carbonyl group that is bonded to the coupling active carbon via an oxygen atom, a nitrogen atom, a sulfur atom, or a carbon atom, a halogen atom, an aromatic azo group, and the like. The aliphatic, aromatic, or heterocyclic group contained in such coupling-off groups may have one or more substituents, as described below.

Examples of coupling-off groups include a halogen atom (e.g., fluorine, chlorine, bromine), an alkoxy group (e.g., ethoxy, dodecyloxy, carboxypropyloxy), an aryloxy group (e.g., 4-chlorophenoxy group, a 4-methoxyphenoxy group), an acyloxy group (e.g., an acetoxy group, a tetradecanoyloxy group), an aliphatic or aromatic sulfonyloxy group (e.g., a methanesulfonyloxy group, a toluenesulfonyloxy group), an acylamino group (e.g., a dichloroacetylamino group, a trifluoroacetylamino group), an aliphatic or aromatic sulfonamido group (e.g., a methanesulfonamido group, a p-toluenesulfonamide group), an alkoxycarbonyloxy group (e.g., an ethoxycarbonyloxy group, a benzyloxycarbonyloxy group), an aryloxycarbonyloxy group (e.g., a phenoxycarbonyloxy group), an aliphatic, aromatic or heterocyclic thio group (e.g., an ethylthio group, a phenylthio group), a carbamoylamino group (e.g., an N-methylcarbamoylamino group, an N-phenylcarbamoylamino group), a 5-membered or 6-membered nitrogen-containing heterocyclic group (e.g., an imidazolyl group, a pyrazolyl group), an imido group (e.g., a succinimido group, a hydantoinyl group), an aromatic azo group (e.g., a phenylazo group), and the like.

The aliphatic, aromatic, or heterocyclic groups included in X and the groups shown by R₁ and R₂ may be substituted by a substituent such as, for example, a halogen atom (e.g., a fluorine atom, a chlorine atom, a bromine atom, etc.), an alkyl group (e.g., a methyl group, a t-octyl group, a dodecyl group, a trifluoromethyl group, etc.), an alkenyl group (e.g., an allyl group, an octadecenyl group, etc.), an aryl group (e.g., a phenyl group, a p-tolyl group, a naphthyl group, etc.), an alkoxy group (e.g., a methoxy group, a benzyloxy group, a methoxyethoxy group, etc.), an aryloxy group (e.g., a phenoxy group, a 2,4-di-tert-amylphenoxy group, a 3-tert-butyl-4-hydroxyphenoxy group, etc.), an acyl group (e.g., an acetyl group, a benzoyl group, etc.), a sulfonyl group (e.g., a methanesulfonyl group, a toluenesulfonyl group, etc.), a carboxy group, a sulfo group, a cyano group, a hydroxy group, an amino group (e.g., a primary amino group, a dimethylamino group, etc.), a carbonamido group (e.g., an acetamido group, a trifluoroacetamido group, a tetradecanamido group, a benzamido group, etc.), a sulfonamido group (e.g., a methanesulfonamido group, a hexadecanesulfonamido group, a p-toluenesulfonamido group, etc.), an acyloxy group (e.g., an acetoxy group, etc.), a sulfonyloxy group (e.g., a methanesulfonyloxy group, etc.), an alkoxycarbonyl group (e.g., a dodecyloxycarbonyl group, etc.), an aryloxycarbonyl group (e.g., phenoxycarbonyl group, etc.), a carbamoyl group (e.g., a dimethylcarbamoyl group, a tetradecylcarbamoyl group, etc.), a sulfamoyl group (e.g., a methylsulfamoyl group, a hexadecylsulfamoyl group, etc.), an imido group (e.g., a succinimido group, a phthalimido group, an octadecenylsuccinimido group, etc.), a heterocyclic group (e.g., a 2-pyridyl group, a 2-furyl group, a 2-thienyl group, etc.), an alkylthio group (e.g., a methylthio group, etc.), and an arylthio group (e.g., a phenylthio group, etc.).

Another useful class of magenta couplers are pyrazoloazole couplers. Pyrazoloazole couplers useful in the practice of the invention include those according to the formula:
wherein
R₃ represents hydrogen or a substituent,
X is as defined above for formula (I), and
Z represents the non-metallic atoms necessary to complete a heterocyclic ring.

A more specific expression of compounds according to formula (II) is made by reference to formula (III):
wherein
R₁ represents hydrogen or a substituent,
X is as described above for formula (I),
Zₐ, Z_{b}, and Z_{c} each represents a substituted or unsubstituted methine group, =N-, or -NH-,
one of either the Zₐ-Z_{b} bond or the Z_{b}-Z_{c} bond is a double bond with the other being a single bond,
when the Z_{b}-Z_{c} bond is a carbon-carbon double bond, it may form part of an aromatic ring, and
when any one of R₁, X, and a substituted methine group represented by Zₐ, Z_{b}, or Z_{c} is a divalent or polyvalent group, it may form a dimer or a polymer.

As the magenta coupler used in the practice of the invention is preferably susceptible to wandering, it will include non-polymeric couplers according to formulas (I) or (II); however, it may also be a polymer, oligomer, or dimer coupler. Such couplers are included in the description of formula (II) above. In the case of formula (I), any of R₁, R₂, or X may also be a divalent or a more polyvalent group to form an oligomer such as a dimer, etc., or may connect a polymeric main chain and a coupler skeleton to form a polymeric coupler. If the magenta coupler is a polymeric coupler, low molecular weight polymer chains or polymer compositions containing unreacted coupler monomer that would exhibit a tendency to wander are preferred. A typical amount of polymeric coupler that would be used in a photographic material will generally represent a number of polymer molecule chains having a distribution of varying molecular weights. The molecular weight of the polymer is usually described as having a single molecular weight, which is actually a mean or average molecular weight around which the actual molecular weights of the molecules are distributed. Thus, some so-called high molecular weight polymeric couplers may contain a sufficient number of low molecular weight molecules so as to make wandering a problem. Such polymeric couplers are intended to be included within the scope of the present invention.

Examples of magenta couplers useful in the practice of the invention are presented below.

The yellow coupler useful in the practice of the invention can be essentially any type of yellow coupler, as is well-known in the art. The reactivity of the yellow coupler with oxidized color developer must be low enough so that, in the absence of the oxidized developer competitor, magenta dye would be formed as a result of reaction between magenta coupler that has wandered out of its layer and developer that has been oxidized by reaction with silver halide from the yellow coupler layer. The selection of a yellow coupler that will benefit from practice of the present invention depends on a number of factors, including the specific magenta coupler involved and its reactivity with oxidized color developer, the choice of oxidized color developer, the concentrations of the yellow and magenta couplers, and other factors affecting the reaction kinetics of oxidized developer and couplers (e.g., pH).

One skilled in the art would know the relative reactivities of yellow couplers in various photographic systems. For example, U.S. Patents 4,710,453, 4,738,917, and 4,820,614, describe relative reactivities of couplers in color negative systems, such as color paper.

The present invention is applicable to color reversal systems, which, unlike color negative systems, do not offer the option of compensating for unwanted magenta dye stain during the printing process. In a preferred embodiment of the invention, the photographic material is a reversal material, such as Kodak Ektachrome® or Fuji Fujichrome®. For a reversal material, the yellow coupler preferably has a relative reactivity, as defined below, of not greater than 0.9.

In this embodiment, the relative reactivity of the yellow coupler is determined as follows. A photographic element is prepared by coating a cellulose acetate-butyrate film support with a photosensitive layer containing 3.77 gm/m² gelatin, 0.76 gm/m² silver bromoiodide emulsion, and 2.7 mmole/m² or the yellow coupler which had been dispersed in half its weight of dibutylphthalate. The photosensitive layer is overcoated with a layer containing gelatin at 1.08 gm/m² and bis-vinyl sulfonyl methyl ether at 1.75 weight percent based upon total gelatin.

The sample is imagewise exposed and processed using Kodak E-6® processing (E-6® processing is described in British Journal of Photography Annual, 1977, pp. 194-197). The relative reactivities represent the status A blue D-max obtained for the sample compared to that obtained for an identical coating, but containing a coupler having the structure:

Examples of yellow couplers useful in the practice of the invention along with their relative reactivity values are presented below.

The oxidized developer competitor compound useful in the practice of the invention has a relative reaction rate of at least 1.6. Such competitor compounds are described as "quencher" compounds in European patent application publication no. 326,406. The relative reaction rate herein considered is what can be determined as a relative value obtainable by measuring the dye density of the color image that coupler N forms after the competitor has been mixed with said coupler, incorporated with a silver halide emulsion, and subjected to color development.
The ratio of reaction activity of a competitor compound with coupler N, represented as R, can be defined in a formula as$\text{R} \text{=} \frac{\text{DM}}{\text{DM′}}$ , wherein DM represents density of a color image of coupler N when a competitor compound is not used; DM′ represents the density of the color image of the coupler N when a competitor compound is added in a quantity of 1/10 mol against coupler N.

The reaction rate of a competitor with the oxidation product of a color developing agent can be determined as a relative value by finding R for the competitor against coupler N in the above formula.

The oxidized developer competitor compound may be incorporated in any layer between the magenta coupler layer and the yellow coupler layer, or within the yellow coupler layer. This layer can be a yellow filter layer, such as a Carey Lea silver layer or a yellow filter dye-containing layer, or it can be a separate interlayer. The effectiveness of the oxidized developer competitor will be felt to a greater extent when the yellow coupler layer and the magenta coupler layer are closer in physical proximity. Thus, preferred embodiments are contemplated when there are no additional silver halide layers between the magenta coupler layer and the competitor layer, between the yellow coupler layer and the competitor layer, or both. The competitor is preferably incorporated in the material at levels of from about 0.03 g/m² to about 0.22 g/m², although other levels may be useful.

An especially preferred class of oxidized developer compounds is described in U.S. Patent 4,923,787. Such compounds have the formula:
wherein
R¹ represents an electron donating group,
R² represents hydrogen, alkyl, alkoxy, aryl, aryloxy, aralkyl or amino of the formula -NHR³, where R³ is phenyl or benzyl, with the proviso that at least one of the substituents R¹ and R² (a) represents (1) a ballast group of sufficient size as to render the hydrazide compound non-diffusible in the photographic element prior to development in alkaline processing solution and (b) comprises a polar group, and
n is 0, 1 or 2.

According to formula (IV), R¹ substituents, which are electron donating groups, include alkyl, which can be substituted or unsubstituted, straight or branched chain, having from 1 to about 20 carbon atoms, preferably from about 8 to about 16 carbon atoms; alkoxy, which can be substituted or an unsubstituted, straight or branched chain, having from 1 to about 20 carbon atoms, preferably from about 8 to about 16 carbon atoms; carboxy; carbonamido having the formula -NR⁴COR⁵; sulfonamido having the -NR⁴SO₂R⁵; or amino having the formula -NR⁴R⁵ where R⁴ is hydrogen or alkyl having from 1 to about 8 carbon atoms and R⁵ is as defined for R⁴ or is a benzyl or a phenyl group which may be substituted.

R² substituents that are alkyl or alkoxy can be as defined for these same substituents in R¹, or R² can be substituted or unsubstituted aryl or substituted or unsubstituted aryloxy having from 6 to about 30 carbon atoms, such as phenyl, phenoxy, naphthyl or naphthoxy.

When R² represents phenyl or phenoxy it is preferred that the aryl ring have a hydrogen bonding substituent in a position ortho to the point of attachment of the carbonyl group to a hydrazide nitrogen atom. Preferred hydrogen bonding groups include hydroxy, primary or secondary amino groups of the formula -NR⁴R⁵, sulfonamido of the formula -NHSO₂R⁴, carbonamido of the formula -NR⁴COR⁵, and ureido of the formula -NHCONHR⁴ where R⁴ and R⁵ can be hydrogen or alkyl of from 1 to about 8 carbon atoms and R⁵ is as defined for R⁴ or a benzyl or phenyl group.

These groups can also be present as substituents on R² alkyl groups or on other positions of R² aryl groups.

A polar group which can represent R¹ or R² can be a single group or a combination of groups which have a π constant which is more negative than -1.0. The π constant is defined by C. Hansch, A.

Leo, S. Unger, K. Hwan Kim, D. Nikaitani and E. T. Lien, in JOURNAL OF ORGANIC CHEMISTRY, 11, 1973 (pp. 1207-1216). The R¹ or R² polar group or groups include, but are not limited to, -NHSO₂CH₃, -NHSO₂aryl,
-CH₂OH, -NH₂, -COOH, -CONH₂, -NHCONH₂, -NHCSNH₂, -N⁺(R⁵)₃, -SO₃⁻, -SO₂⁻ and
These groups tend to increase the surfactant nature of the hydrazine during alkaline processing.

The alkyl, alkoxy, aryl, aryloxy, aralkyl and benzyl groups which are represented by one or more of R¹, R², R³, R⁴ and R⁵ can be substituted with halogen atoms, for example chlorine, or with haloalkyl groups, for example trifluoromethyl, or with -NO₂ , -CN,

Examples of oxidized developer competitor compounds useful in the practice of the invention are disclosed in the above-referenced EP 326,406 and U.S. 4,923,787, and include:

The support of the element of the invention can be any of a number of well-known supports for photographic elements. These include polymeric films such as cellulose esters (e.g., cellulose triacetate and diacetate) and polyesters of dibasic aromatic carboxylic acids with divalent alcohols (e.g., poly(ethylene terephthalate)), paper, and polymer-coated paper. Such supports are described in further detail in Research Disclosure, December, 1989, Item 308119 [hereinafter referred to as Research Disclosure I], Section XVII.

The silver halide emulsion used in the practice of the invention can contain, for example, silver bromide, silver chloride, silver iodide, silver chlorobromide, silver chloroiodide, silver bromoiodide, or mixtures thereof. The emulsions can include coarse, medium, or fine silver halide grains bounded by 100, 111, or 110 crystal planes. Silver halide emulsions and their preparation are further described in Research Disclosure I, Section I. Also useful are tabular grain silver halide emulsions, as described in Research Disclosure, January, 1983, Item 22534 and U.S. Patent 4,425,426.

The couplers and competitor compound described above used in the practice of the invention (and other couplers and compounds contained in the photographic material) can be incorporated in hydrophilic layers of photographic materials by techniques well-known in the art. One common technique involves the use of high-boiling water-immiscible organic solvents and/or surfactants. Useful organic solvents include tricresyl phosphates, di-n-butyl phthalate, and others described in Research Disclosure I, Section XIV. Surfactants are well-known to one skilled in the art, and are described in Research Disclosure I, Section XI. Mixtures of solvents and surfactants may also be used.

The silver halide described above can be sensitized to a particular wavelength range of radiation, such as the red, blue, or green portions of the visible spectrum, or to other wavelength ranges, such as ultraviolet, infrared, and the like. In a preferred embodiment, the silver halide emulsion associated with the magenta coupler is spectrally sensitized to green light so as to complement the magenta color of the dye formed by the coupler during processing. The silver halide emulsion associated with the yellow coupler is preferably spectrally sensitized to blue light so as to complement the yellow color of the dye formed by the coupler. Chemical sensitization of silver halide can be accomplished with chemical sensitizers such as gold compounds, iridium compounds, or other group VIII metal compounds. Spectral sensitization is accomplished with spectral sensitizing dyes such as cyanine dyes, merocyanine dyes, styryls, or other known spectral sensitizers. Additional information on sensitization of silver halide is described in Research Disclosure I, Sections I-IV.

Although only a yellow coupler layer and a magenta coupler layer are required for the practice of the invention, multicolor photographic elements generally comprise a blue-sensitive silver halide layer having a yellow color-forming coupler associated therewith, a green-sensitive layer having a magenta color-forming coupler associated therewith, and a red-sensitive silver halide layer having a cyan color-forming coupler associated therewith. The oxidized developer competitor compound can be incorporated in the yellow coupler layer or, more preferably, in an interlayer between the yellow coupler layer and the magenta coupler layer. This interlayer can be the yellow filter layer typically used in color photographic materials between the yellow and magenta layers, or it can be a separate layer. Color photographic elements and color-forming couplers are well-known in the art and are further described in Research Disclosure I, Section VII.

The element of the invention can also include any of a number of other well-known additives and layers, as described in Research Disclosure I. These include, for example, optical brighteners, antifoggants, oxidized developer scavengers (which can be the same as or different than the competitor according to formula (I)), development accelerators, image stabilizers, light-absorbing materials such as filter layers or intergrain absorbers, light-scattering materials, gelatin hardeners, coating aids and various surfactants, overcoat layers, interlayers and barrier layers, antistatic layers, plasticizers and lubricants, matting agents, development inhibitor-releasing couplers, bleach accelerator-releasing couplers, and other additives and layers known in the art.

The photographic elements of the invention, when exposed, are processed to yield an image. Processing can be by any type of known photographic processing, as described in Research Disclosure I, Sections XIX-XXIV. A negative image can be developed by color development with a chromogenic developing agent followed by bleaching and fixing. A positive image can be developed by first developing with a non-chromogenic developer, then uniformly fogging the element, and then developing with a chromogenic developer.

Bleaching and fixing can be performed with any of the materials known to be used for that purpose. Bleach baths generally comprise an aqueous solution of an oxidizing agent such as water soluble salts and complexes of iron (III) (e.g., potassium ferricyanide, ferric chloride, ammonium or potassium salts of ferric ethylenediaminetetraacetic acid), water-soluble persulfates (e.g., potassium, sodium, or ammonium persulfate), water-soluble dichromates (e.g., potassium, sodium, and lithium dichromate), and the like. Fixing baths generally comprise an aqueous solution of compounds that form soluble salts with silver ions, such as sodium thiosulfate, ammonium thiosulfate, potassium thiocyanate, sodium thiocyanate, thiourea, and the like.

The invention is further illustrated by the following Example.

On a cellulose triacetate film support provided with a subbing layer was coated each layer having the composition set forth below to prepare a multilayer color photographic light-sensitive material which was designated sample 101.

In the composition of the layers, the coating amounts are shown as g/m² except for sensitizing dyes, which are shown as the molar amount per mole of silver halide present in the same layer.
First Layer: Anithalation Layer
Second Layer: Intermediate Layer
Third Layer: Slow Red Sensitive Layer
Fourth Layer: Fast Red Sensitive Layer
Fifth Layer: Intermediate Layer
Sixth Layer: Slow Green Sensitive Layer
Seventh Layer: Fast Green Sensitive Layer
Eighth Layer: Yellow Filter Layer
Ninth Layer: Blue Sensitive Layer
Tenth Layer: First Protective Layer
Eleventh Layer: Second Protective Layer

Samples 102 to 106 were prepared in the same manner as described above for Sample 101 except for the addition of the competitors listed in Table I to the Eighth Layer. The added competitors were coated at the levels (in g/m²) shown in Table I.

Each of the samples thus prepared was cut into a 35mm width strip. The samples were exposed to a step exposure using green and red light followed by a series of blue flash exposures and processed using standard Kodak E-6® processing solutions and methods. The Status A green density was measured (or interpolated) for an area in the reversal D-min region of the step exposure of each sample with a Status A blue density of 3.0. These values are tabulated in Table I; higher values indicate an increased amount of magenta dye formed by magenta coupler which has migrated out of its layer. The degree of coupler which has migrated out of its layer. The degree of coupler wandering was confirmed by photomicrography.

From the results shown in Table I above, it is clear that the samples using competitors selected according to the present invention effectively suppress the unwanted formation of dye from magenta coupler which has migrated out of its layer. The competitors selected according to the invention offered an advantage over the comparison competitor even when the comparison competitor was coated at twice the level of the competitor selected according to the invention.

The components employed for the preparation of the light-sensitive materials not already identified above are shown below.
Sensitizing Dye-1
Sensitizing Dye-2
Sensitizing Dye-3
Solvent 1 - tritolyl phosphates
Solvent-2 - dibutyl phthalate
Dye-1
Dye-2
Competitor A

The invention has been described in detail with particular reference to preferred embodiments thereof, but it will be understood that variations and modifications can be effected within the spirit and scope of the invention.

## Claims

1. A color reversal photographic material comprising a support having thereon:
a magenta coupler layer that includes a silver halide emulsion and a magenta coupler compound,
a yellow coupler layer that includes a silver halide emulsion and a yellow coupler compound,
characterized in that:
the magenta coupler compound is one that is susceptible to wandering out of the layer in which it is coated,
the yellow coupler compound has a relative reactivity of not greater than 0.9, and
the yellow coupler layer, or a layer between it and the magenta coupler layer, includes an oxidized developer competitor compound having a relative reaction rate of at least 1.6, wherein
the relative reactivity of the yellow coupler can be determined by preparing a photographic element which is imagewise exposed and processed, the relative reactivity being the status A blue D-max obtained for the photographic element compared to that obtained for an identical coating, but containing a coupler having the structure: and the relative reaction rate of the oxidized developer competitor compound can be determined by measuring the dye density of the color image that coupler N forms after the competitor has been mixed with said coupler, incorporated with a silver halide emulsion, and subjected to color development, the relative reaction rate of the competitor compound being defined as the ratio of the density of a color image of coupler N when a competitor compound is not used to the density of the color image of the coupler N when a competitor compound is added.

2. A color reversal photographic material according to claim 1, further characterized in that the magenta coupler compound is a 5-pyrazolone which has the formula: wherein
R₁ represents a carbonamido group, an arylamino group, a ureido group, a sulfonamido group, an alkylamino group, or a heterocyclic amino group,
R₂ represents a substituted or unsubstituted aryl group, and
X represents hydrogen or a group capable of being released by a coupling reaction with an oxidized aromatic primary amine developing agent.

3. A color reversal photographic material according to claim 2, further characterized in that the oxidized developer competitor compound has the structure: wherein
R¹ represents an electron donating group,
R² represents a hydrogen, alkyl, alkoxy, aryl, aryloxy, aralkyl or amino of the formula -NHR³, where R³ is phenyl or benzyl, with the proviso that at least one of the substituents R¹ and R² (a) represents a ballast group of sufficient size as to render the hydrazide compound non-diffusible in the photographic element prior to development in alkaline processing solution and (b) comprises a polar group, and
n is 0, 1 or 2.

4. A color reversal photographic material according to claim 3, further characterized in that, if n is 1 or 2, then R¹ is carbonamido of the formula -NR⁴COR⁵ where R⁴ is hydrogen or alkyl of 1 to 8 carbon atoms and R⁵ is as defined for R⁴ or a benzyl or phenyl group.

5. A color reversal photographic material according to any of claims 1 thru 4, further characterized in that the yellow coupler has a relative reaction rate of not greater than 0.8 and the oxidized developer competitor compound has a relative reaction rate of at least 1.7.

6. A color reversal photographic material according to any of claims 1 thru 5, further characterized in that the yellow coupler layer is nearer to the magenta coupler layer than any other yellow coupler layer in the material.

7. A color reversal photographic material according to any of claims 1 thru 6, further characterized in that the magenta coupler layer is nearer to the yellow coupler layer than any other magenta coupler layer in the material.

8. A color reversal photographic material according to any of claims 1 thru 7, further characterized in that the layer containing the oxidized developer competitor is also a yellow filter layer.

9. A color reversal photographic material according to any of claims 1 thru 7, further characterized in that the layer containing the oxidized developer competitor is other than a yellow filter layer.

10. A color reversal photographic material according to any of claims 1 thru 7, further characterized in that the oxidized developer competitor is contained in the yellow coupler layer.

## Patentansprüche

1. Photographisches Farbumkehrmaterial mit einem Träger, auf dem sich befinden:
eine Purpurrot-Kuppler-Schicht, die eine Silberhalogenidemulsion und eine Purpurrot-Kupplerverbindung enthält,
eine Gelb-Kuppler-Schicht, die eine Silberhalogenidemulsion und eine Gelb-Kupplerverbindung enthält,
dadurch gekennzeichnet, daß:
die Purpurrot-Kupplerverbindung eine solche ist, die für eine Auswanderung aus der Schicht, in der sie aufgetragen ist, zugänglich ist,
die Gelb-Kupplerverbindung eine relative Reaktivität von nicht größer als 0,9 aufweist, und
die Gelb-Kuppler-Schicht oder eine Schicht zwischen dieser und der Purpurrot-Kuppler-Schicht eine Mitbewerberverbindung für oxidierten Entwickler enthält, die eine relative Reaktionsgeschwindigkeit von mindestens 1,6 aufweist, wobei
die relative Reaktivität des Gelb-Kupplers bestimmt werden kann durch Herstellung eines photographischen Elementes, das bildweise exponiert und entwickelt wird, wobei die relative Reaktivität der D-max-Wert für Status-A-Blau ist, erhalten für das photographische Element im Vergleich zu dem Wert, der im Falle einer identischen Beschichtung, jedoch mit einem Kuppler der folgenden Struktur: erhalten wird,
und wobei die relative Reaktionsgeschwindigkeit der Mitbewerberverbindung für oxidierten Entwickler bestimmt werden kann durch Messung der Farbstoffdichte des Farbbildes, das der Kuppler N bildet, nachdem die Mitbewerberverbindung mit dem Kuppler vermischt worden ist, in eine Silberhalogenidemulsion eingearbeitet und einer Farbentwicklung unterworfen wurde, wobei die relative Reaktionsgeschwindigkeit der Mitbewerberverbindung definiert ist als das Verhältnis der Dichte eines Farbbildes des Kupplers N, wenn eine Mitbewerberverbindung nicht verwendet wird, zur Dichte des Farbbildes des Kupplers N, wenn eine Mitbewerberverbindung zugesetzt wird, wobei der Kuppler N der folgenden Formel entspricht:

2. Photographisches Farbumkehrmaterial nach Anspruch 1, weiter dadurch gekennzeichnet, daß die Purpurrot-Kupplerverbindung ein 5-Pyrazolon ist, das der Formel entspricht: worin bedeuten:
R₁ eine Carbonamidogruppe, eine Arylaminogruppe, eine Ureidogruppe, eine Sulfonamidogruppe, eine Alkylaminogruppe oder eine heterocyclische Aminogruppe,
R₂ eine substituierte oder unsubstituierte Arylgruppe, und
X ein Wasserstoffatom oder eine Gruppe, die durch eine Kupplungsreaktion mit einer oxidierten, aus einem primären aromatischen Amin bestehenden Entwicklerverbindung freigesetzt wird.

3. Photographisches Farbumkehrmaterial nach Anspruch 2, weiter dadurch gekennzeichnet, daß die Mitbewerberverbindung für oxidierten Entwickler die folgende Struktur hat: worin bedeuten:
R¹ eine Elektronen spendende Gruppe,
R² gleich Wasserstoff, Alkyl, Alkoxy, Aryl, Aryloxy, Aralkyl oder Amino der Formel -NHR³, worin R³ für Phenyl oder Benzyl steht, wobei gilt, daß mindestens einer der Substituenten R¹ und R² (a) eine Ballastgruppe einer ausreichenden Größe ist, um die Hydrazidverbindung in dem photographischen Element vor der Entwicklung in alkalischer Entwicklungslösung nicht-diffundierend zu machen und (b) eine polare Gruppe aufweist, und
n gleich 0, 1 oder 2.

4. Photographisches Farbumkehrmaterial nach Anspruch 3, weiter dadurch gekennzeichnet, daß, falls n gleich 1 oder 2 ist, dann R¹ eine Carbonamidogruppe der Formel -NR⁴COR⁵ ist, worin R⁴ steht für Wasserstoff oder Alkyl mit 1 bis 8 Kohlenstoffatomen, und worin R⁵ wie R⁴ definiert ist oder eine Benzyl- oder Phenylgruppe ist.

5. Photographisches Farbumkehrmaterial nach einem der Ansprüche 1 bis 4, weiter dadurch gekennzeichnet, daß der Gelb-Kuppler eine relative Reaktionsgeschwindigkeit von nicht größer als 0,8 hat, und daß die Mitbewerberverbindung für oxidierten Entwickler eine relative Reaktionsgeschwindigkeit von mindestens 1,7 hat.

6. Photographisches Farbumkehrmaterial nach einem der Ansprüche 1 bis 5, weiter dadurch gekennzeichnet, daß die Gelb-Kuppler-Schicht näher der Purpurrot-Kuppler-Schicht liegt als jede andere Gelb-Kuppler-Schicht in dem Material.

7. Photographisches Farbumkehrmaterial nach einem der Ansprüche 1 bis 6, weiter dadurch gekennzeichnet, daß die Purpurrot-Kuppler-Schicht näher der Gelb-Kuppler-Schicht liegt als irgendeine andere Purpurrot-Kuppler-Schicht in dem Material.

8. Photographisches Farbumkehrmaterial nach einem der Ansprüche 1 bis 7, weiter dadurch gekennzeichnet, daß die Schicht, die die Mitbewerberverbindung für oxidierten Entwickler enthält, ferner eine Gelbfilterschicht ist.

9. Photographisches Farbumkehrmaterial nach einem der Ansprüche 1 bis 7, weiter dadurch gekennzeichnet, daß die Schicht, die die Mitbewerberverbindung für oxidierten Entwickler enthält, eine andere Schicht als eine Gelbfilterschicht ist.

10. Photographisches Farbumkehrmaterial nach einem der Ansprüche 1 bis 7, weiter dadurch gekennzeichnet, daß der Mitbewerber für oxidierten Entwickler in der Gelb-Kuppler-Schicht vorhanden ist.

## Revendications

1. Produit photographique inversible en couleurs comprenant un support recouvert :
d'une couche de coupleur magenta comprenant une émulsion aux halogénures d'argent et un composé coupleur magenta,
d'une couche de coupleur jaune comprenant une émulsion aux halogénures d'argent et un composé coupleur jaune,
caractérisé en ce que :
le composé coupleur magenta est celui qui est susceptible de migrer hors de la couche dans laquelle il est appliqué,
le composé coupleur jaune a une réactivité relative qui n'est pas supérieure à 0,9 et
la couche de coupleur jaune, ou une couche placée entre cette couche et la couche de coupleur magenta comprend un composé concurrent du développateur oxydé ayant une vitesse relative de réaction d'au moins 1,6,
et la réactivité relative du coupleur jaune peut être déterminée en préparant un produit photographique qui est exposé conformément à l'image et traité, la réactivité relative étant la D-max Status A dans le bleu obtenue pour le produit photographique comparée à celle obtenue avec un couchage identique, mais contenant un coupleur de formule : et la vitesse de réaction relative du composé concurrent du développateur oxydé est déterminée en mesurant la densité de colorant de l'image colorée que le coupleur N forme après que le composé concurrent a été mélangé au coupleur, incorporé dans l'émulsion aux halogénures d'argent et soumis à un développement chromogène, la vitesse de réaction relative du composé concurrent étant définie comme le rapport de la densité d'image de colorant du coupleur N quand un composé concurrent n'est pas utilisé à la densité de l'image de colorant du coupleur N quand un composé concurrent est rajouté de formule :

2. Produit photographique inversible en couleurs selon la revendication 1 caractérisé en ce que le composé coupleur magenta est une 5-pyrazolone de formule : où
R₁ représente un groupe carbonamido, arylamino, uréido, sulfonamido, alkylamino ou hétérocyclique amino,
R₂ représente un groupe aryle substitué ou non, et
X représente l'hydrogène ou un groupe capable d'être libéré par une réaction de couplage avec un développateur amine primaire aromatique oxydé.

3. Produit photographique inversible en couleurs selon la revendication 2 dans lequel le composé concurrent du développateur oxydé a la formule : où
R¹ représente un groupe donneur d'électrons,
R² représente l'hydrogène, un groupe alkyle, alkoxy, aryle, aryloxy, aralkyle ou amino de formule -NHR³, où R³ est phényle ou benzyle, avec la condition qu'au moins l'un des substituants R¹ et R² (a) représente un groupe ballast de taille suffisante pour rendre le composé hydrazide non-diffusible dans l'élément photographique avant le développement dans la solution alcaline de traitement et (b) comprend un groupe polaire, et
n est 0,1 ou 2.

4. Produit photographique inversible en couleurs selon la revendication 3 dans lequel si n est 1 ou 2, R¹ est carbonamido de formule NR⁴COR⁵ où R⁴ est l'hydrogène ou alkyle de 1 à 8 atomes et R⁵ est tel que défini pour R⁴ ou un groupe benzyle ou phényle.

5. Produit photographique inversible en couleurs selon les revendications 1 à 4 dans lequel le coupleur jaune a une vitesse de réaction relative, qui n'est pas supérieure à 0,8 et le composé concurrent du développateur oxydé a une vitesse de réaction relative d'au moins 1,7.

6. Produit photographique inversible en couleurs selon les revendications 1 à 5 dans lequel la couche de coupleur jaune est plus proche de la couche de coupleur magenta que toute autre couche de coupleur jaune dans le produit.

7. Produit photographique inversible en couleurs selon les revendications 1 à 6 dans lequel la couche de coupleur magenta est plus proche de la couche de coupleur jaune que toute autre couche de coupleur magenta dans le produit.

8. Produit photographique en couleurs selon les revendications 1 à 7 dans lequel la couche contenant le composé concurrent du développateur oxydé est aussi une couche filtre jaune.

9. Produit photographique en couleurs selon les revendications 1 à 7 dans lequel la couche contenant le composé concurrent du développateur oxydé est autre qu'une couche filtre jaune.

10. Produit photographique en couleurs selon les revendications 1 à 7 dans lequel le composé concurrent du développateur oxydé est contenu dans la couche de coupleur jaune.
